

W. B. MOORE.

## PROCESS IN MAGNETIC SEPARATION.

APPLICATION FILED AUG. 31, 1906.

922,800.

Patented May 25, 1909.



### Witnesses

Wm. M. Haenel  
Gas & Water

၃၃၄

Adams & Brooks

Attorneys

# UNITED STATES PATENT OFFICE.

WALTER B. MOORE, OF SEATTLE, WASHINGTON.

## PROCESS IN MAGNETIC SEPARATION.

No. 922,800.

Specification of Letters Patent.

Patented May 25, 1909.

Application filed August 31, 1906. Serial No. 332,869.

*To all whom it may concern:*

Be it known that I, WALTER B. MOORE, a citizen of the United States of America, and a resident of the city of Seattle, in the county 5 of King and State of Washington, have invented certain new and useful Improvements in Processes in Magnetic Separation, of which the following is a specification.

My invention relates to an improved 10 method of treating finely divided materials carrying magnetic particles or magnetite for the purpose of separating the magnetic from the non-magnetic particles.

The invention has special reference to the 15 treatment of sand or gangue containing magnetic iron in a granular or pulverulent form for the purpose of separating from the mass the magnetic constituent.

The primary object of my invention is to 20 rapidly and economically recover all, or practically all, of the magnetic particles combined in masses of material of the class mentioned.

It is also my object not only to rapidly 25 recover the magnetic constituent but also to readily concentrate the same free from all non-magnetic particles.

In carrying out my invention, the materials mixed with water to flow freely, are 30 directed to pass in suspension in the magnetic field of a magnetic separating means in which an electro-magnet of suitable strength operates to attract and hold all of the magnetic particles or magnetite to a 35 shield, while such of the non-magnetic particles not caught in magnetic entanglements are carried away by the water. As fast as magnetic particles are extracted from the mass of materials they are subjected to 40 magnetic force directed to cause the particles to leave the magnetic separating means and pass across an air gap or passage-way. This may be accomplished by employing permeable means acting in the magnetic field of 45 the electro-magnet to concentrate lines of force and operating the shield of said magnet continuously to convey the particles drawn thereto into the field of force of said means. To concentrate the magnetic particles free 50 from the non-magnetic matter carried therewith in magnetic entanglements the particles are subjected to a rapid reversal of magnetic polarity to cause them to travel end over end, as they clear the air gap or passage-way, to 55 and across suitable supporting means. It is preferable that the magnetic particles should

be kept constantly in a wet state throughout the process and for this purpose water may be caused to flow upon the particles as they pass from the magnetic separating means 60 upon the support.

In the accompanying drawing there is disclosed one form of apparatus devised and constructed by me to carry out the above described process, said apparatus forming 65 the subject of my application for patent on magnetic separators prepared and executed by me on even date herewith.

With reference to the drawing, Figure 1 is a vertical transverse section of the apparatus, and Fig. 2 is a side elevation of the same viewed from the right of Fig. 1 portions of some of the parts being broken away.

The magnetic separating means, as shown, comprises an electro-magnet 1, and a cylindrical shield 2, the former of which in operation, is connected with a suitable electrical energizer in any convenient manner. The magnet is secured to a shaft 3 which fits rotatably in suitable hubs on the shield and is 80 supported in a frame 4 for rotation. Secured to the shaft and shield are pulleys 5 and 5' respectively to which power is applied to rotate the magnet and shield independently of each other. 85

Reference numeral 6 indicates a conduit communicating with a chamber 7, which embraces the lower portion of shield 2, and is provided with a discharge passage 8.

In the magnetic field, at the upwardly 90 moving side of magnet 1 are permeable members 9 which are close to but not in contact with shield 2, and adjacent these members are jet tubes 10 which are connected with a suitable delivery pipe and arranged to direct 95 water for discharge toward respective members 9. Extending, each from its respective member 9, are supports 12, 12 and 12' the latter of which is provided with an upwardly inclined extension 14 and an opening at the 100 base of said extension which communicates with a valve 15.

In operation the materials mixed with water are passed through conduit 6 into chamber 7 where the magnetic particles are drawn by magnet 1 to the shield 2, while the non-magnetizable matter overflows into the discharge passage 8. As fast as the magnetic particles are extracted and drawn to the shield, they are carried into the field of force of the lower member 9 to which they fly and by rapid reversal of polarity, effected 110

by the rotation of magnet 1, they are immediately caused to travel end over end to and across support 12'. If the shield should be overloaded with magnetic materials, a part 5 thereof will be conveyed beyond the lower member and removed by the succeeding members 9. Particles passing to said last members are immediately caused to travel to and across respective supports 12. During 10 the end over end movements of the particles, such non-magnetic matter as may be carried therewith in magnetic entanglements will be freed and gravitate to the base of the extension 14, while the magnetic particles falling from the supports 12 will be caught on said extension and travel across the same in company with those particles passing from support 12', to a trough or receptacle 17.

Having 20 thus described my invention, what I claim as new, and desire to secure by Letters Patent of the United States of America, is:—

1. The process of recovering magnetic particles 25 associated with non-magnetic materials, which consists in feeding the mass of materials into a magnetic field, subjecting the particles retained in the field to an opposing magnetic force to move them across a 30 passage-way, and then subjecting the parti-

cles to a rapid reversal of magnetic polarity to cause them to travel end over end.

2. The process of recovering magnetic particles 35 associated with non-magnetic materials, which consists in feeding the mass of materials into a magnetic field to extract the magnetic particles from the remainder, conveying the extracted magnetic particles, magnetically impelling the extracted particles across a passage-way, directing a fluid 40 on said particles and subjecting them to a rapid reversal of magnetic polarity to cause them to turn end over end.

3. The herein described process which consists in feeding the mass of materials into a 45 magnetic field to extract the magnetic particles from the remainder, impelling the extracted magnetic particles across a passage-way, then subjecting the magnetic particles to a rapid reversal of magnetic polarity to 50 cause them to turn end over end, and directing water on said magnetic particles while they are turning end over end.

Signed at Seattle, Washington this 23 day of August 1906.

WALTER B. MOORE.

Witnesses:

JOHN W. FILKINS,  
S. B. FOLEY.